

## UNITED STATES PATENT OFFICE.

KOJIRO KAWAMURA, OF TOKYO-FU, JAPAN, ASSIGNOR OF ONE-HALF TO YOSHIMATSU YOKOYAMA, OF KANAZAWA, JAPAN.

## DIFFERENTIAL-FLOTATION PROCESS FOR MIXED SULPHIDE ORES.

No drawing.

Application filed January 18, 1926. Serial No. 82,125.

My invention relates to the differential flotation process characterized in that anhydrous cromic acid is used in the flotation process to separate the mixed sulphide ore containing several sulphide minerals, e. g. iron pyrite, chalco-pyrite, zinc blend, etc., the action of anhydrous cromic acid effecting to stop provisionally the floatage of chalco-pyrite and iron-pyrite, while zinc blend alone floats up beforehand; has for its object the economical differential separation of the valuable minerals contained. But, when the impure anhydrous cromic acid common in the market is to be used for this object, it has to be mixed up with proper quantity of the alkaline salts, for it usually contains sulphuric acid more or less. The quantity of added alkali must be in such a proportion that the sulphuric acid present is neutralized; this must be found by test to prevent an over-addition of alkali which would form bichromate salts with the chromic acid present.

My invention consists in the process in which chalco-pyrite and zinc blend are separated and picked out respectively and very economically out of the mixed sulphide ore, which hitherto existing processes, the dressing or the flotation, have been unable to attain. For example, the result of the differential flotation process, hitherto commonly known reagents being used, is as the following Table No. I.

Table No. I.

|              | Amount of ore | Grade |          |          | Extraction |          |          |          |
|--------------|---------------|-------|----------|----------|------------|----------|----------|----------|
|              |               | Gr.   | Cu       | Fe       | Zn         | Amount   | Cu       | Fe       |
| Original ore |               |       | Per cent | Per cent | Per cent   | Per cent | Per cent | Per cent |
| Concentrate  | 400           | 9.13  | 24.77    | 29.43    |            | 100.00   | 100.00   | 100.00   |
| Middling     | 137.8         | 2.08  | 3.86     | 57.62    |            | 34.45    | 7.86     | 5.37     |
| Tailing      | 11.1          | 9.60  | 17.01    | 32.61    |            | 8.27     | 8.71     | 5.68     |
|              | 229.1         | 13.30 | 38.48    | 3.81     |            | 57.28    | 83.43    | 88.95    |

In the existing flotation process, as illustrated in the above table, zinc blend floats up always with the other sulphide minerals so that these valuable minerals could not be economically separated. Moreover, in the other existing differential flotation process in which a certain chemical, or chemicals, is, or are, used as the reagent, the floatage of iron pyrite is provisionally somewhat stopped, while most of the chalco-

pyrite, being affected comparatively little, float up with zinc blend and so that the chalco-pyrite can not separate economically with zinc blend. In the case of my present process, however, anhydrous cromic acid being used as the reagent, not only the floatage of iron pyrite is provisionally stopped, but also that of chalco-pyrite is very much affected as compared within the case of hitherto known reagents being used, and eventually the amount of chalco-pyrite mixed in the floating zinc blend is so little that the economical separation between zinc blend and chalco-pyrite is carried out almost perfectly. One of the experimental results in the process is as the following Table No. II.

Table No. II.

|              | Amount of ore | Grade |          |          | Extraction |          |          |          |
|--------------|---------------|-------|----------|----------|------------|----------|----------|----------|
|              |               | Gr.   | Cu       | Fe       | Zn         | Amount   | Cu       | Fe       |
|              |               |       | Per cent | Per cent | Per cent   | Per cent | Per cent | Per cent |
| Original ore | 400           | 9.13  | 24.77    | 29.43    |            | 100.00   | 100.00   | 100.00   |
| Concentrate  | 137.8         | 2.08  | 3.86     | 57.62    |            | 34.45    | 7.86     | 5.37     |
| Middling     | 11.1          | 9.60  | 17.01    | 32.61    |            | 8.27     | 8.71     | 5.68     |
| Tailing      | 229.1         | 13.30 | 38.48    | 3.81     |            | 57.28    | 83.43    | 88.95    |

In the above table, the middling is to be treated again being placed back into the original ore, at the practical operation. As illustrated in the above table, if anhydrous aromatic acid is used as the reagent, both chalco-pyrite and iron pyrite are affected very much and their floatage is stopped almost entirely, while most of the zinc blend being affected little floats up into the concentrated mineral, resulting in the ratios of zinc grade 57.62% and extraction percent 80.27%. The present invention hereby succeeds in the separation and picking out between chalco-pyrite and zinc blend almost to a perfect degree, which have hitherto been taken for almost impossible. Anhydrous cromic acid to be used for this object, extends from  $\frac{1}{100}$  to  $\frac{1}{100.00}$  against that of the original ore.

When galena is also contained in the original ore it is understood that the separation is carried out by the process of specific gravity concentration.

I claim:—

The process of differentially floating ores comprising adding crude commercial anhydrous chromic acid with alkali to neutralize sulphuric acid therein to a pulp containing a mixture of sulphide minerals, said chromic acid being added in quantity sufficient to inhibit flotation of cupriferous

and ferric sulphides without affecting zinc sulphide, and then subjecting the mixture to flotation. <sup>10</sup>

In testimony whereof, I have hereunto set my hand.

KOJIRO KAWAMURA.